# EUROPEAN PATENT SPECIFICATION

(11) **EP 1 108 507 B1**
(45) Date of publication and mention of the grant of the patent: **03.11.2010**
(21) Application number: 00670010.8
(22) Date of filing: 13.11.2000
(51) Int. Cl.: B27K 7/00, A62D 3/00

(54) **Method of solid-liquid extraction applied to cork products**
Verfahren zur Fest-Flüssig-Extraktion, angewendet bei Korkprodukten
Procédé d'extraction solide-liquide aplliquée à des produits en liège

(30) Priority: 16.11.1999 PT 10237699
(43) Date of publication of application: 20.06.2001
(73) Proprietor: Amorim & Irmaos S.A., 4535 Santa Maria de Lamas Codex (PT)
(72) Inventor: Leal Ferreira, José Manuel, 4535 Santa Maria de Lamas Codex (PT)
(74) Representative: Alves Moreira, Pedro

(56) References cited:
- FR-A- 343 350
- FR-A- 384 559
- GB-A- 267 733
- GB-A- 1 604 803
- US-A- 3 560 251

## Description

### 1 - OBJECT OF INVENTION

The invention relates to the decontamination of cork products by means of a solid-liquid extraction method based on the successive application of pressure changes on a liquid surface in which the cork is immersed, which causes cork contraction and expansion, thereby causing the release of contaminants entrapped within the cork.

### 2 - STATE OF THE ART

Cork is a natural porous product that contains in its surface, and within it, a variety of contaminants derived from its life experience in the forest which, when in contact with liquids, can cause organoleptic changes in those liquids.

During the last years, a variety of methods have been developed and applied in an attempt to eliminate said contaminants. The existing methods are based on the immersion of cork in disinfectant baths, alternate with centrifugation steps. Due to the operating conditions, these methods do not eliminate all contaminants, namely those entrapped within the cork, which can, subsequently originate organoleptic changes in the liquids with which the cork product will contact.

*In 1993 it was patented (*PT 101215 of 1993.03.11*) a thermochemical process for the expansion of cork using a pressurised system (relative pressure from 9,8 to 29.4 bars) where cork is immersed in the presence of some organic solvents, namely methanol, ethanol, formic acid, dichloromethane or chloroform*.

*Although some features of the above patent are similar to those of the present invention, its subject-matter is different as it aims to achieve cork material expansion which is not related with decontamination.*

*It was found that water is an appropriate liquid to be used in the decontamination process, which constitutes an advantage in view of its availability with a substantial reduction in the final cost of the decontamination process*.

### 3 - DETAILED DESCRIPTION OF THE INVENTION

The applicant has found that this problem of incomplete decontamination of cork products could be solved through an hydrodynamic method through which the cork to be treated is put in an airtight recipient and, subsequently, immersed **in water that should be placed at a temperature ranging from 20°C to 200°C.**

Then, a relative pressure of up to 10 bar is applied on the surface of the liquid, for 1 to 3600 seconds, using any kind of gas or gas mixture. Then, the gas is released until the recipient pressure reaches the atmospheric pressure again. Thereafter the pressure is reduced by means of an appropriate vacuum pump until a relative pressure of up to -1 bar is reached. After being under this reduced pressure for 1 to 3600 seconds the system is caused to return to the atmospheric pressure.

These cycles of differential pressure are repeated several times until the desired cork purity is reached. A simple experimentation will set the number of cycles required.

Those skilled in the art will understand that changes can be made to the method of the invention, which should be understood, as being encompassed within the scope of the appended claims.

## Claims

1. Method of solid-liquid extraction applied to cork products for the decontamination thereof, **characterised in that** it comprises the following steps:
a. Putting the cork product in a airtight recipient,
b. Filling the airtight recipient with water so that the cork product is completely immersed **in that** liquid,
c. Applying a relative pressure of up to 10 bar on the liquid surface, for 1 to 3600 seconds, using an appropriate gas,
d. Releasing the pressurising gas until the pressure within the recipient reaches atmospheric pressure,
e. Reducing the pressure within the recipient, by means of an appropriate vacuum pump, until a relative pressure of up to -1 bar is reached, during a time period of 1 to 3600 seconds,
f. Causing the recipient to return to atmospheric pressure.

2. Method according to the preceding claims **characterised in that** the gas used to apply pressure on the surface of the decontamination liquid is air, a gas different from air or a gas mixture.

3. Method according to the preceding claims **characterised in that** the treatment cycle is repeated up to 100 times.

## Patentansprüche

1. Verfahren von Fest-Flüssig-Extraktion, das auf Korkerzeugnisse für die Entseuchung davon verwendet wird, **dadurch gekennzeichnet, dass** es die folgenden Schritte umfasst:
a. Das Korkerzeugnis in einen luftdichtem Behälter stellen,
b. Den luftdichten Behälter mit Wasser füllen, so dass das Korkerzeugnis in dieser Flüssigkeit ganz eingetaucht wird,
c. Einen verhältnismäßigen Druck von bis zu 10 bar auf dem Flüssigkeitsspiegel während 1 bis 3600 Sekunden anwenden, wobei ein geeignetes Gas verwendet wird,
d. Das Unterdruckgas abgeben, bis der Druck innerhalb des Behälters den Luftdruck erreicht,
e. Den Druck innerhalb des Behälters mittels einer geeigneten Vakuumpumpe verringern, bis ein verhältnismäßiger Druck von bis zu 1 bar während einer Zeitdauerr von 1 bis 3600 Sekunden erreicht wird,
f. Veranlassen dass de Behälter zum Luftdruck zurückkehret.

2. Verfahren nach dem vorhergehenden Anspruch, **dadurch gekennzeichnet, dass** das für die Druckanbringung auf dem Spiegel der entseuchenden Flüssigkeit verwendete Gas Luft, ein Gas, das nidht als Luft ist, oder eine Gasmischung ist.

3. Verfahren nach einem der vorhergehenden Ansprüche, **dadurch gekennzeichnet, dass** der Behandlungsablauf bis zu 100 mal wiederholt wird.

## Revendications

1. Méthode d'extraction solide-liquide appliquée à des produits en liège pour leur décontamination, **caractérisée en ce qu'**elle comprend les phases suivantes:
a. Mise du produit en liège dans un récipient étanche à l'air,
b. Remplissage du récipient étanche à l'air avec de l'eau, de telle façon que le produit en liège est complètement immergé dans ce liquide-là,
c. Application d'une pression relative de jusqu'à 10 bar sur la surface du liquide pendant 1 à 3600 secondes, en employant un gaz adéquat,
d. Dégagement du gaz pressurisé jusqu'à ce que la pression à l'intérieur du récipient atteint la pression atmosphérique,
e. Réduction de la pression à l'intérieur du récipient, à l'aide d'une pompe à vide adéquate, jusqu'à atteindre une pression relative de jusqu'à 1 bar, pendant une durée de 1 à 3600 secondes,
f. Laisser le récipient revenir à la pression atmosphérique.

2. Méthode selon la revendication précédente, **caractérisée en ce que** le gaz pressurisé employé pour appliquer de la pression sur la surface du liquide de décontamination est l'air, un gaz autre que l'air ou un mélange de gaz.

3. Méthode selon les revendications précédentes, **caractérisée en ce que** le cycle de traitement est répété jusqu'à 100 fois.
